

# UNITED STATES PATENT OFFICE.

LEONARD LORENTOWICZ, OF IRVINGTON, NEW JERSEY.

## METHOD FOR THE ELIMINATION OF WASTEFUL DISCARDING OR THROWING ASIDE OF DEFECTIVE METAL CASTINGS.

1,246,444.

Specification of Letters Patent. Patented Nov. 13, 1917.

No Drawing.

Application filed March 6, 1917. Serial No. 152,882.

To all whom it may concern:

Be it known that I, LEONARD LORENTOWICZ, citizen of the United States, residing at Irvington, Essex county, New Jersey, have invented certain new and useful Improvements in Methods for the Elimination of Wasteful Discarding or Throwing Aside of Defective Metal Castings, of which the following is a specification.

10. The invention relates to improvements in methods for the elimination of wasteful discarding or throwing aside of defective metal castings, and more particularly such castings as are used in the manufacture of engine cylinders.

Heretofore, in the art of making castings, enormous wastefulness has been necessary due to the presence of holes or openings, commonly known as "pores", in the walls 20 thereof, and which are generally of such area or depth as to render the same unfit for use.

Attempts have been made to render these defective castings usable, but in the majority of instances the same have proven very unsuccessful. One of the best known methods employed for the purpose has been to subject that portion of the casting, adjacent the opening or pore, to a heat sufficient to melt the metal and allow it, when molten, to fill 30 the opening, and then harden therein, but, in so doing, it has been found that the casting has been otherwise injured and ruined by the warping of the same out of its normal shape.

35. The primary object of the invention is to provide a method of filling the openings or pores in castings, and one wherein the latter is in no way injured during the filling operation.

40. Another object of the invention is to provide a filling for the carrying out of the method aforesaid, and one which is capable of being readily applied for the purpose-mentioned, and which, when properly applied, becomes firmly incorporated in the casting and may be subjected to any reasonable degree of heat without being effected by the same when in use.

With these and other objects in view, the 50 invention resides in the certain new and useful method as will be hereinafter more fully described, and set forth in the appended claims.

In carrying out the present invention, 55 when a casting is found to be defective with

one or more openings or pores therein, it is first desired that the openings or pores be thoroughly cleared of the usual outer metallic crust and of any other foreign matter therein, and for this purpose, it is contemplated to use a bur or reamer, preferably one of a power driven type involving a driven flexible shaft to facilitate the use of the same from any angle necessary to perform the work. The walls of the opening or pore are now treated with a suitable acid, and a flux, to destroy all effects of oxidation thereon, and to allow for a thorough adhering there-to of the metallic filling to be applied to the same.

This metallic filling may be of any desired metal, preferably reduced to a finely divided state, and after the opening or pore has been filled with the same, it is to be subjected to an arc or spot flame, so that it is thoroughly fused. While in heated condition, the filling is now thoroughly pressed into the opening or pore, and is subjected to a rubbing action by means of relatively heavy irons, which may be in the form of soldering irons having relatively heavy heads of either copper or nickel, and which may be, and preferably are heated during the pressing or rubbing operation.

The surplus metal of the filling is now to be scraped off, and the surface of the same reduced to conform to the contour of the finished surface in which it is embedded, and for this purpose, it is contemplated to use implements involving scraper blades of various shapes and sizes to conform to the contour of the finished surface of a casting.

In the treating of castings to be subjected to high temperatures, such as the castings of the cylinders of internal combustion engines, it is desired that the metallic filling be of a metal, or a combination of metals, having a relatively high temperature coefficient, and it has been found that babbitt is admirably suited for the present purpose, the same being used alone, or in conjunction with either one, or all, of such metals, as copper, nickel, and silver, in proportions of approximately two per cent. (2%) of the latter metals.

From the foregoing, it will be readily obvious that the invention provides for a marked saving in the various manufactures of articles from castings, such as has heretofore been rendered impossible by reason of

losses due to a large percentage of the castings being imperfect to such a degree as to necessitate their being discarded and laid aside, and afterward remelted for subsequent recasting.

Having thus fully described the invention, what is claimed, is:—

1. The method of making usable defective castings, which consists in cleaning out the pores therein, subjecting the walls of the pores to the action of an acid, and applying a flux thereto, filling the pores with a metallic substance, subjecting the filling to the action of localized heat, subjecting the filling, while in heated condition, to pressure and rubbing the same into a homogeneous state, and finally scraping away the surplus of the filling and reducing the latter

to conform to the contour of the finished surface of the casting.

2. The method of making usable defective castings, which consists in cleaning out the pores therein, subjecting the walls of the pores to the action of an acid, and applying a flux thereto, filling the pores with a metallic compound, subjecting the filling to the action of an arc or spot flame, subjecting the filling, while in fused state, to pressure and rubbing the same into a homogeneous state, and finally scraping away the surplus of the filling and reducing the latter to conform to the contour of the finished surface of the casting.

In testimony whereof I affix my signature.

LEONARD LORENTOWICZ.